

## UNITED STATES PATENT OFFICE

1,983,450

DELUSTERED RAYON AND SPINNING  
SOLUTION THEREFOR

Frank H. Griffin, Wawa, Pa., assignor to The  
Viscose Company, Marcus Hook, Pa., a corpora-  
tion of Pennsylvania

No Drawing. Application September 29, 1932,  
Serial No. 634,078

2 Claims. (Cl. 106—40)

This invention consists of a process of produc-  
ing delustered rayon, and the delustered rayon  
so produced.

It has been proposed to deluster rayon yarn  
5 by the use of titanium dioxide, but the use of this  
delustrant carries the objection that it gives to  
the yarn a peculiar shiny appearance. This ap-  
pearance may be characterized as metallic, par-  
ticularly when such yarn is dyed with the deeper  
10 shades. For example, the blues tend to show a  
kind of coppery appearance, particularly when  
viewed in sunlight at certain angles. This phe-  
nomenon has been one of the chief objections to  
the use of this method of delustering rayon.

15 I have found that this disadvantage of the  
use of titanium dioxide may be eliminated by  
the use of a delustrant consisting of the combi-  
nation of chlorinated diphenyl with titanium di-  
oxide. This chlorinated diphenyl (commercially  
20 known as aroclor) is itself a delustrant, and adds  
to the delustering effect of the titanium dioxide,  
as well as eliminating the peculiar shiny appear-  
ance which results from the use of titanium alone.

The amounts may vary between 0.1 to 5.0 per-  
25 cent titanium dioxide and between 0.5 to 15.0  
percent chlorinated diphenyl. A preferred ex-  
ample of yarn produced by my invention is one  
containing 0.6 percent titanium dioxide and 4.5  
percent chlorinated diphenyl. This preferred ex-  
30 ample is as dull as a yarn containing 1.3 percent  
titanium dioxide, but does not have its undesir-  
able metallic appearance. The percentages given  
herein are based on the weight of the cellulosic  
content of the viscose solution, or by weight dry  
35 yarn. Naturally the proportions might be varied  
somewhat in response to the preference of cus-  
tomers, but as a rule the amount of aroclor used  
will always greatly exceed the amount of tita-  
nium dioxide.

40 The required amounts of titanium dioxide and  
chlorinated diphenyl in finely divided form, either  
separately or together, are distributed through-

out the solution to be spun, prior to the spinning  
thereof. The required amount of finely divided  
titanium dioxide is thoroughly mixed with a  
small amount of water and a dispersing agent,  
such as, Turkey red oil. Similarly the required  
amount of finely divided solid aroclor is thor-  
oughly mixed with water and dispersing agent.  
The two delustrants might be prepared together  
in a mixed suspension. These suspensions, either  
singly or together, are added to the solvent used  
to dissolve the cellulose xanthate or preferably  
are added to the cellulose xanthate solution just  
prior to completion of the solution operation.  
The xanthate solution containing delustrants is  
then filtered, aged, de-aerated, and spun in the  
normal manner. It is, of course, possible to add  
the delustrant to the xanthate solution after the  
filtering and aging but prior to the spinning.

45 After the titanium dioxide and chlorinated di-  
phenyl are incorporated into the solution as de-  
scribed above, the solution is spun in the usual  
manner.

I claim:—

1. Viscose solution adapted to be spun into de-  
lustered rayon yarn and containing from about  
50 0.1 to 5.0 per cent titanium dioxide delustrant and  
from about 0.5 to 15.0 per cent chlorinated di-  
phenyl delustrant, the percentages being based on  
the weight of the cellulosic content of the viscose  
solution, the amount of chlorinated diphenyl pres-  
55 ent being substantially in excess of the amount of  
titanium dioxide, and both delustrants being  
in the form of finely divided solid particles.

2. As a new article of manufacture, delustered  
rayon containing from about 0.1 to 5.0 per cent  
60 titanium dioxide delustrant and from about 0.5  
to 15.0 per cent chlorinated diphenyl delustrant,  
by weight of the dry yarn, the amount of chlori-  
nated diphenyl present being substantially in  
excess of the amount of titanium dioxide. 65

FRANK H. GRIFFIN.